

April 28, 1931.

H. M. GERSMAN

1,802,811

METHOD OF EXPANDING METAL

Filed April 30, 1926



INVENTOR  
Harvey M. Gersman  
BY  
App and Powers.  
ATTORNEY

## UNITED STATES PATENT OFFICE

HARVEY M. GERSMAN, OF BUFFALO, NEW YORK

## METHOD OF EXPANDING METAL

Application filed April 30, 1926. Serial No. 105,722.

This invention relates to a method of expanding metal and proposes a method by which the expanded article has the same length as the blank from which it is produced and the expansion is effected in connection with the elongation of the strands and bonds. The invention is generically applicable to the production of expanded metal articles of different kinds and for different uses in structural operations, and is herein claimed in its generic aspect and also in one specific aspect, namely, the production of expanded metal beams or load bearing members.

The principal objects of the invention are to enable the production of expanded metal articles in forms which are highly advantageous by reason of their structural features and physical characteristics and qualities and which cannot be satisfactorily produced by methods heretofore employed or proposed, and to provide a method which, along with these advantages, may be carried out in connection with standard rolling practice as utilized for the production of the blank, which may be practiced at relatively low cost, and which is especially conformable to the peculiar conditions under which the work is done, that is to say, the rapid travel of the blank and its rapid cooling.

The invention is practiced in connection with a heated rolled blank and the method is completed before the blank has cooled to a degree sufficient to interfere with the working of the metal. Preferably the invention is practiced continuously with the delivery of the blank from a standard mill pass and the method is commenced with the blank at or near the degree of heat which it has at the delivery stage of the rolling operation.

According to the invention the heated blank is first suitably slit and its expansion is then effected by rolling a portion of the blank in which the slits are incorporated, the rolled portion being thereby reduced in thickness and increased in length, and during the elongation of the rolled portion which occurs after and results from the rolling operation simultaneously and progres-

sively increasing the width of the blank between unelongated portions at each side of the rolled portion, thereby simultaneously to compensate and continuously take up the elongation of the rolled portion at a rate corresponding to that of the elongation and with resultant expansion of the blank. The increase in the width of the blank between the unelongated portions may be effected in different ways. As shown it is effected by spreading or fanning out the unelongated portions. The method is thus one in which no warping or buckling of the metal is produced or permitted and in which there are no factors by which inequalities in form or physical characteristics are introduced or by which, as compared with cold expanding operations, any internal stresses are developed. It follows that the product is one in which the elongated strands and bonds are uniform in thickness, dimensions and physical qualities and may lie in planes coincident with the mean or general plane of the expanded article.

As applied to load bearing members the web is slit and by the subsequent rolling elongated while the flanges remain of the same length as in the blank and during the elongation of the web are simultaneously and progressively and at a rate proportionate to the elongation spread or fanned out so as to compensate or take up the elongation as it occurs and with resultant expansion of the blank into the load bearing member which is desired, although this is not necessary, may be passed through finishing rolls.

The above and other characterizing features of the method will be set forth as the description proceeds and will appear from the accompanying drawing which illustrates apparatus by which the method may be practiced, the steps in the evolution of the blank into the completed product, and a portion of an expanded beam produced by the method.

In said drawing:

Figure 1 is a plan view of the apparatus, showing the blank in its different stages of treatment.

Figure 2 is a longitudinal sectional view of the same.

Figure 3 is a fragmentary perspective view of one of the rolls which reduce and elongate the slitted portion of the blank.

Figure 4 is a plan view of a portion of the expanded beam.

Figure 5 is a section on the line 5—5 of Figure 4.

The method is preferably practiced continuously and in connection with the rolling of the blank. In such case the heat of blank as it comes from the stand of the mill by which its development has been brought to the stage desired is utilized and the method is completed with final determination of the form and physical qualities of the expanded article while the blank is yet sufficiently hot for its parts to be worked and relocated.

The method is applicable to different forms of beams and other expanded articles and is herein illustrated in connection with the production of a beam in the form of a simple lattice truss wherein the struts have a single line of intermediate bonds representing points of intersection, the remaining bonds being the connections between the struts and the chords, that is to say, the panel points of the truss. The blank for such a beam will have parallel slits arranged in three longitudinal rows with the slits of each row in alignment and staggered relatively to the slits of the adjacent row or rows, the relative length and arrangement of the slits being such as to provide for the symmetrical relation of the bonds and the struts by making due allowance for the elongation of the bonds in the expanded product.

The blank B is shown as having a cross section similar to that of a standard I-beam and is provided with parallel flanges 1 and a web 2. The blank may be delivered from a standard mill pass (not shown) and is first acted upon by slitting rolls 3 which slit the web. These rolls may be of any suitable construction and are merely shown diagrammatically.

The web having thus been slit in any usual or suitable manner, the blank is now ready for reduction and expansion. These operations may be performed in one stage or in more than one stage according to the degree of reduction and expansion desired, it being practical to continue the expansion to a point where the struts associated with each chord extend at approximate angles of 60 degrees to one another. Two stages of reduction and expansion are shown in the drawing.

From the slitting rolls the blank passes to reducing rolls 4 which act on the slitted portion of the web and reduce its thickness with consequent elongation. The slitted portion

of the web which has been acted on by the reducing rolls will, owing to the elongation, travel at a greater rate than that of the blank as it passes through the slitting rolls, the increase in speed being proportionate to the percentage of reduction.

For example, if the speed of the blank up to the reducing rolls be 100 feet per minute the speed of the web upon passing from the reducing rolls may be approximately 120 feet per minute.

For practical reasons the reduction in any one pair of rolls is limited to substantially twenty-five percent and where greater reduction is required additional rolls are necessary. The reducing rolls are employed in cooperation with means for increasing the width of the blank simultaneously and continuously with the resultant elongation and at a rate proportionate to that of the elongation.

In the embodiment disclosed such means is constituted by shoes 5 which act on the flanges. These shoes are preferably provided in upper and lower pairs, one pair being associated with each reducing roll and the shoes of each pair having forwardly divergent guide faces 6 which bear against the inner faces of the flanges 1, the inclination of the faces 6 being determined in accordance with the requirements previously stated, that is to say, to effect the spreading or fanning out of the flanges so as to continuously compensate or take up the elongation simultaneously and at a rate proportionate to its progress with resultant formation of the reduced and elongated part of the web into open work.

The shoes 5 preferably engage the flanges substantially at or slightly ahead of the center line of the rolls whereby they commence to act on the flanges substantially at the time when reducing pressure is applied to the slitted portions of the blank. Under such pressure there is a tendency for the parts to widen very slightly and the initial action of the shoes 5 is, therefore, to prevent any welding or "freezing" of the reduced portions along the sides of the slits prior to expansion and thereby to insure that during expansion no stresses are imposed on the panel point bond providing portions such as might arise if it were necessary to separate any adjacent strands which had become partially welded.

It will be noted that the spreading or fanning out of the flanges is not resorted to for the purpose of elongating the struts and has no effect on the length of the struts but is resorted to for the purpose of compensating or taking up the elongation of the struts as it progresses, and accomplishes this result by causing the struts to have a lateral travel or deflection which with respect to the length of the beam equalizes their elongation. The formation of the rolled portion of the web into open work is thus accomplished simultaneously with the elongation of the struts.

taneously and at a proportionate rate to the elongation of the struts and the bonds.

Any tendency for the struts in consequence of their elongation to shear or partially shear from the adjacent chord portions may be counteracted in various ways. As herein shown this is accomplished by forming the reducing rolls whereby they will not act on the bonds which connect the struts and chord portions. Thus the reducing rolls are formed adjacent their margins with recesses or flats 7 of suitable outline, preferably triangular outline and which are arranged at such intervals as to coincide with the panel point bond portions of the blank. The result of the provision of the recesses or flats 7 is that the said panel point bond portions are not rolled and hence are not reduced and elongated but remain of their original thickness. It follows that substantially triangular reenforced panel points are provided and that the reduction and elongation of the struts are confined to rectangular areas which said panel points adjoin. If a second stage of expansion be required, as is assumed by the drawing, this is effected by reducing rolls 8 and shoes 9 which are duplicates in structure and arrangement of the rolls 4 and shoes 5. The rolls 8 act on the web as it passes from the shoes 5 and carry the reduction and elongation to a further degree and the shoes 9 act on the flanges 2 in the same manner as the shoes 5 and carry the expansion to a corresponding further degree.

Having fully described my invention, I claim:

1. The method of expanding metal which is practiced with a heated slitted blank and which consists in reducing and thereby elongating a part of said blank in which slits are incorporated without elongating adjacent parts and increasing the width of the blank at the beginning and during the progress of the elongation and at a proportionate rate, thereby continuously to compensate and take up the elongation at a rate proportionate to its progress.

2. The method of expanding metal which is practiced with a heated slitted blank and which consists in reducing and thereby elongating a part of said blank in which slits are incorporated without elongating adjacent parts and spreading or fanning out the said unelongated adjacent parts at the beginning and during the progress of the elongation of the reduced parts and at a rate proportionate to the rate of elongation, thereby continuously to compensate and take up the elongation as it progresses.

3. The method of expanding metal which is practiced with a heated blank having a slitted portion and unslitted portions at each side of the slitted portion and which consists in reducing and thereby elongating the slitted portion and at the beginning and

during the progress of such elongation acting on the unslitted portions to increase the width of the blank at a rate proportionate to that of the elongation, thereby continuously to compensate and take up the elongation as it progresses.

4. The method of expanding metal which is practiced with a heated blank having a slitted portion and unslitted portions at each side of the slitted portion and which consists in reducing and thereby elongating the slitted portion and at the beginning and during the progress of such elongation and at a proportionate rate spreading or fanning out the unslitted portions, thereby continuously to compensate and take up the elongation as it progresses.

5. The method of expanding metal which is practiced with a heated blank having a slitted portion and which consists in reducing and thereby elongating the slitted portion and at the beginning and during the progress of the elongation and at a proportionate rate spreading or fanning out the unelongated portions at each side of the slitted portion, thereby continuously to compensate and take up the elongation as it progresses.

6. The method of expanding metal which is practiced with a heated slitted blank and which consists in reducing and thereby elongating a part of said blank in which slits are incorporated without elongating adjacent parts and causing a lateral travel or deflection of the reduced parts at the beginning and during the progress of their elongation and at a proportionate rate by which such elongation is equalized with respect to the length of the blank.

7. The method of making an expanded load bearing member from a heated flanged rolled blank which consists in slitting the web of the blank, rolling the slitted web to reduce and elongate it without altering the length of the flanges, and acting on the flanges at the beginning and during the progress of the elongation of the rolled web and at a proportionate rate whereby to increase the width of the blank, and to compensate and take up the elongation as it progresses.

8. The method of making an expanded load bearing member from a heated flanged rolled blank which consists in slitting the web of the blank, rolling the slitted web to reduce and elongate it without altering the length of the flanges and spreading or fanning out the flanges at the beginning and during the progress of the elongation of the rolled web and at a proportionate rate whereby to increase the width of the blank and to compensate and take up the elongation as it progresses.

9. The method of making an expanded load bearing member from a heated flanged

rolled blank which consists in slitting the web of the blank in parallel rows to provide for struts and panel points in the finished beam, rolling the slitted web to reduce and elongate it without altering the length of the flanges and in a manner to counteract any shearing tendency at the panel points in consequence of the elongation, and acting on the flanges at the beginning and during the progress of the elongation of the rolled web and at a proportionate rate whereby to increase the width of the blank and to compensate and take up the elongation as it progresses.

15 10. The method of making an expanded load bearing member from a heated flanged rolled blank which consists in slitting the web of the blank in parallel rows to provide for struts and panel points in the finished beam, rolling the slitted web to reduce and elongate it without rolling the panel points and without altering the length of the flanges, and acting on the flanges at the beginning and during the progress of the elongation of the rolled web and at a proportionate rate whereby to increase the width of the blank and to compensate and take up the elongation as it progresses.

11. The method of expanding metal which is practiced with a heated blank and which consists in rolling a slitted portion of said blank between parallel non-slitted portions thereof thereby to elongate the slitted portion relatively to the unslitted portions and commencing at the center of the roll pass and continuing throughout the elongation of the slitted portion gradually increasing the relative spacing of the non-slitted portions to counteract buckling of the rolled portion during its elongation and at the same time bring the rolled portion into flat expanded condition.

In testimony whereof I affix my signature.  
HARVEY M. GERSMAN.

45

50

55

60

65